

A. A. LOCKWOOD,  
TREATMENT OF COPPER ORES.  
APPLICATION FILED JAN. 20, 1917.

1,262,892.

Patented Oct. 29, 1918.

Fig. 1.



Fig. 2.



Inventor,  
Alfred Andrew Lockwood  
By his attorney  
Baldwin Wright

# UNITED STATES PATENT OFFICE.

ALFRED ANDREW LOCKWOOD, OF FOREST HILL, ENGLAND.

## TREATMENT OF COPPER ORES.

1,282,892.

Specification of Letters Patent.

Patented Oct. 29, 1918.

Application filed January 20, 1917. Serial No. 143,479.

To all whom it may concern:

Be it known that I, ALFRED ANDREW LOCKWOOD, a subject of the King of Great Britain, residing at 55 Kilmorie road, Forest Hill, in the county of Surrey, England, have invented a new and useful Improvement in the Treatment of Copper Ores, of which the following is a specification.

This invention relates to a process by which copper may be precipitated directly from a pulped ore without filtration.

According to my invention I lead copper pulp from a preparatory vessel, provided with agitating means, into a precipitating vessel containing depending electrodes, and pass a current through the acid pulp kept in suspension by a jet of air, means being also provided for leading back the residue of pulp to the preparatory vessel, after the electrolytic operation.

The cathodes which I prefer to employ consist of iron plates coated with an easily removable skin of copper. The copper skin is rendered easily removable by first coating the plates with a layer of carbon (which term is intended to include graphite, or a carbonaceous material such as tar) and then depositing a copper coating upon the plates in any convenient manner.

As, moreover, carbon coated iron cathodes during electrolysis of a pulped copper ore become quickly coated with a copper skin, the cathode plates may in the first stages of the electrolysis consist of iron plates coated with tar or other adhesive carbonaceous material, or with graphite. When a graphite coated iron plate is employed the graphite must be made to adhere to the plate by some adhesive material such as varnish or tar.

The finely ground ore previously mixed with water or with an acid leaching solution (in either case so as to produce an acid pulp) is led into an open vessel having a series of anodes which may be of lead, and a series of the special cathodes hung from supports at the top, and a low tension current is passed between them. The current employed will necessarily depend upon the ore used. With a roasted sulfid ore, in the form of a pulp containing  $\frac{1}{2}\%$  of free  $H_2SO_4$  at the time the same enters the electrolytic vat, I have employed a current of about 2 volts, and about .25 amperes per square foot of cathode area. With other

ores, larger or smaller amounts of acid, and higher or lower current densities, can be used.

The series of anodes and cathodes are so arranged that only a small interval (about one inch) is left between each anode and cathode for the passage of the pulp.

In some cases the ore may contain a sufficient quantity of acid radical for example  $SO_4$ , but if it does not there is introduced into the pulp either before it is led into the precipitating vessel or when it is in the vessel, either at the commencement of the electrolysis or during the progress thereof, acid as required.

The invention is illustrated in the accompanying drawings, in which Figure 1 is a side elevation of the plant and Fig. 2 is a plan of the precipitating vessel.

In the drawings *a* is the open precipitating vessel with depending electrodes *a*<sup>1</sup> and an air inlet pipe *a*<sup>2</sup> for maintaining the ore in suspension.

*b* is a vessel containing pulp which flows through a pipe *c* into the vessel *a* and from thence is pumped back to the top of the vessel *b* through a pipe *d*.

*e* is a pipe through which air is delivered for maintaining the ore in suspension.

The cathode which I prefer to employ in the process, is constructed as follows:

The iron plates are dipped into boiling tar and then covered with powdered graphite, these operations being repeated as many times as is necessary, and in some cases there is deposited upon the graphite coating a skin of copper, or a skin of copper is deposited upon the tarred plate, omitting the graphite.

Care should be taken that the coating of graphite and the copper skin should be continuous and free from air bubbles.

At the conclusion of the electrolysis the copper deposited upon the cathodes may be readily removed by warming them and then stripping off the copper.

With electrodes thus prepared the difficulty that is sometimes met with in the treatment of copper ores containing iron where the cathodes are apt to be attacked by ferric and ferrous oxids produced during electrolysis is not experienced.

The agitation of the acid pulp in the vessel *b* aids solution of a part of the copper content of the ore, until the liquor contains

- an amount of dissolved copper capable of being efficiently extracted by electrolysis. Solution of the copper is also aided by the aeration. The pulp, without filtration, flows 5 to the electrolytic vat *a*, and in this vessel the current causes the deposition of copper on the cathodes, which acid is formed at the anodes. This acid, in its nascent state, is highly active, and at once attacks copper in 10 the suspended ore, dissolving a part of the same, forming copper salts which may be electrolyzed. This action continues until the pulp is passed back to the vessel *b*, where the returned pulp mixes with the other pulp 15 therein, the acid thus coming into contact with a less completely leached ore than that returned in the pulp from vessel *a*. This free acid will act upon more of the copper ore in the pulp in vessel *b*. During the entire cyclic passage of the ore from *b*, through 20 *c*, *a*, pump and *d* back to *b*, there is no filtering step, and no sedimenting step, the purpose being to maintain an effective suspension 25 of the ore particles in the leaching liquor, throughout the process. The circulation is continued until the copper content of the ore under treatment falls to a very low figure, practically no copper being left in the treated ore.
- 30 For a more complete explanation, it may be stated that with sulfid ores, it is advisable to roast the ore, so that the copper is largely in the form of sulfate, and the iron in the form of insoluble oxid. Carbonate ores may 35 sometimes be advantageously roasted, but this is usually unnecessary. The vessel *b* may be filled about half to two-thirds full of fine ore, and an acid liquor, *e.g.*, diluted sulfuric acid added to nearly fill the vessel.
- 40 The air blast is then introduced at *e*, until a fairly complete mixture ensues, and the liquid pulp then allowed to pass to the vessel *a*, air being introduced at *a'*, and the pump started. The amount of acid in the liquor 45 added should be sufficient to leave the pulp acid. The liquor flowing through *d* into *b* is, of course, more strongly acid than the liquor flowing out through *c*.
- What I claim is:—
- 50 1. A process of electro-depositing copper which comprises first forming a bulk of an

acid pulp containing copper ore material in a liquid, agitating and aerating the said pulp, by air injected thereinto, leading pulp carrying matter in suspension therein into 55 an electrolytic vessel and passing an electrolytic current from an insoluble anode through the pulp to a cathode to deposit copper on the latter, while preventing sedimentation of the insoluble material of said pulp 60 by introducing air into the lower part of the liquid, and returning the so treated pulp to the bulk of acid pulp, and repeating the cycle of operations.

2. A process of recovering copper from 65 copper ores which comprises producing an acid ore pulp by aerating and agitating a bulk of copper ore material with a suitable aqueous liquid, continuing the agitation by aeration of the pulp while withdrawing a 70 constant current of said acid ore pulp to an electrolytic bath having vertical insoluble electrodes therein, agitating the pulp in said electrolytic bath by the introduction of air at the lower part thereof, while passing an 75 electric current through said bath to deposit copper, and continuously passing the treated pulp back from said electrolytic bath to said bulk of acid pulp, all without settling or filtration of the acid pulp at any stage of the 80 cyclic process.

3. A process for treating copper ores which consists in agitating the pulped ore in a preparatory vessel, leading the agitated pulp from this vessel into a precipitating vessel 85 containing depending insoluble anodes and iron cathodes, subjecting the pulp in the precipitating vessel to electrolysis whereby copper is deposited at the cathodes and simultaneously maintaining the pulp in a condition 90 of agitation therein.

4. A process for treating copper ores which consists in agitating the pulped ore in a preparatory vessel, leading the agitated pulp from this vessel into a precipitating vessel 95 containing depending insoluble anodes and iron cathodes, subjecting the pulp in the precipitating vessel to the action of an electric current and simultaneously maintaining the same in suspension therein.

ALFRED ANDREW LOCKWOOD.